

## UNITED STATES PATENT OFFICE

2,364,790

## TREATMENT OF ORGANIC DIELECTRIC MATERIALS WITH HIGH-FREQUENCY ELECTRIC CURRENT

Charles B. Hemming, Parlin, N. J., assignor to E. I. du Pont de Nemours & Company, Wilmington, Del., a corporation of Delaware

No Drawing. Application September 13, 1941,  
Serial No. 410,785

7 Claims. (Cl. 204—165)

This invention relates to the application of high frequency electrostatic fields to organic substantially non-conducting materials and more particularly to a means for increasing the electrical losses of such materials when exposed to high frequency electrostatic fields.

A unique method for joining a plurality of parts by exposing a thermo-sensitive adhesive having relatively high hysteresis characteristics to high frequency electrostatic field is described in U. S. Patent 2,087,480. It was found that sufficient heating occurs to soften or fuse or otherwise affect the adhesive to cause bonding. Previously heat had been applied through conduction by hot pressure plates, ovens or other external heat sources. Dependent upon the heat conductivity of the parts to be joined, the time necessary to secure satisfactory joints was often long and seriously delayed manufacturing operations. As suggested in the patent, it is characteristic of the action of high frequency fields that uniform and rapid heating of the materials exposed occurs, that is, absorption of electrical energy occurs throughout the materials, limited only by the hysteresis characteristics of the materials exposed. Excessive surface heating is, therefore, avoided, and the time required to heat thick objects is substantially the same as for thin objects.

It has been found advantageous to use electrical frequencies in the more commonly used radio frequency range of 100,000 cycles to 100 megacycles per second. The voltage applied may be varied over wide ranges but in general an input voltage of at least 1000 is necessary in commercial practice.

The process is particularly adaptable to the cementing of the component parts of shoes, for the manufacture of plywood, for cementing cork granules and many other cementing operations. The process is particularly advantageous where the materials to be joined are non-metallic and are poor conductors of heat. It is a characteristic of the electrostatic field that in the radio frequency range very little electrical energy is absorbed by metallic conductors. The system is, therefore, adapted to organic polymeric materials which are ordinarily considered to be good dielectrics for direct or low frequency alternating currents, that is, materials having dielectric constants of 20 or less at 60 cycles.

It is generally assumed that the extent of the hysteresis loss of a material can be expressed comparative to those of other materials by comparing the products of the dielectric constant

times the power factor. The larger the product of these constants, the greater is the energy absorption from a radio frequency field. For example, polystyrene with a dielectric constant of 5 and a power factor of 0.0001 (at 60 cycles) has as its product a value of 0.00025. Methyl methacrylate with a dielectric constant of 3.5 and a power factor of 0.06 has as its product the value 0.21 or one over 800 times as great as styrene. 10 In an electrostatic field having a frequency of 30 megacycles per second and an impressed voltage of 2000, methyl methacrylate heats readily while polystyrene is practically unaffected. It is important as a result of this fact to develop 15 means for modifying the more perfect dielectrics so that they will heat readily and quickly in the radio frequency fields.

It is an object of this invention to provide a means of controlling the absorption of electrical 20 energy by organic polymeric materials, particularly thermoplastic, organic resinous dielectrics at radio frequencies. A further object is the provision of a means of increasing the energy absorption by the more perfect dielectrics. A 25 still further object is the provision of modifiers for organic polymeric materials which do not greatly alter the physical properties of the compositions. Other objects will appear hereinafter.

I have found that titanium dioxide in its rutile 30 and brookite crystalline forms has electrical properties such that although it represents a very efficient dielectric alone at radio frequencies, it acts in an unexpected manner when incorporated in substantially non-conducting organic compositions and gives blended compositions of greater hysteresis characteristics than represented by the titanium dioxide free material.

Titanium dioxide is known in three crystalline forms: rutile, brookite, and anatase. The heating 40 of brookite and anatase above 820° C. tends to convert them to the rutile form. All three forms possess high dielectric constants, with those of rutile and brookite having the very abnormal dielectric constants of approximately 114 and 78, 45 respectively. The anatase form shows a dielectric constant of 31. The high dielectric constants are coupled with very low power factors, so that the product of the dielectric constant times the power factor is low. The tendency of 50 the rutile to absorb electrical energy from a radio frequency field is slight, and the material can be used as an insulator in these fields.

Unexpectedly, however, when finely divided rutile or brookite is incorporated into a polymeric organic material, the hysteresis losses of

the mixture become greater than those of either the titanium dioxide or the organic materials alone. The effect is applicable to a considerable variety of compositions based upon film forming polymeric organic materials. The increase in hysteresis losses through the incorporation of the finely divided titanium dioxide means that electrostatic fields of lower intensities can be used to obtain the required degree of heating or at any workable intensity a more rapid heating will be obtained. In many cases adhesives which cannot be made to heat satisfactorily in the available electrostatic fields can be modified with the rutile or brookite to produce materials which can be activated.

The following examples are given by way of illustration and no limitations are intended thereby except as indicated in the present invention:

*Example 1*

|                         | Percent by weight |
|-------------------------|-------------------|
| Polyvinyl butyral resin | 18.7              |
| DLbutyl phthalate       | 9.4               |
| Denatured ethyl alcohol | 36.3              |
| Toluol                  | 35.6              |
|                         | 100.0             |

This example was compared in heating characteristics in a radio frequency field of 2000 volts at 30 megacycles per second, with the same composition in which 34% by weight of the total solids content of finely divided rutile had been incorporated by rapid mixing. Both compositions were applied by brushing to the rough side of 1 x 6 inch strips of shoe sole leather and allowed to dry  $\frac{1}{2}$  hour at 60° C.

A second coat was then applied and dried for  $\frac{1}{2}$  hour at 60° C. following which they were allowed to stand for 4 hours in a room at 24.5° C. Heating tests were then carried out using a treater input voltage of 2100 at a frequency of 30 megacycles. The electrostatic field was set up between two adjustable metal plates, between which the leather samples were placed in the same plane. As the initial test, two uncoated leather strips were placed between the treater plates for 45 seconds. The temperature of the strips at the end of the treatment was obtained by inserting a quick-acting metallic thermometer of the Weston type between the strips before any appreciable heat could be dissipated through the leather. The strips coated with the unmodified adhesive composition were tested under the same electrical conditions and finally the strips coated with the adhesive containing the rutile were similarly tested. The following averaged results were obtained:

|                            | Temperature reached | Rise above room temperature |
|----------------------------|---------------------|-----------------------------|
| Leather strips—no adhesive | 65                  | 40                          |
| Leather+adhesive           | 71                  | 46                          |
| Leather+adhesive+rutile    | 75                  | 50                          |

Longer periods of treatment gave higher temperature rises but of a comparable order of difference. Excellent bonds were secured with the adhesive containing the rutile modifier.

*Example 2*

|                           | Percent by weight |
|---------------------------|-------------------|
| Ethyl cellulose           | 18.7              |
| DLbutyl phthalate         | 9.4               |
| Ethyl alcohol (denatured) | 36.2              |
| Toluol                    | 35.7              |
|                           | 100.0             |

10 66.2 parts by weight of this composition were mixed with 33.8 parts by weight of rutile and the mixture applied by brushing two coats on four 1" x 6" sole leather strips. Similarly, two coats 15 of the unmodified composition were applied to four other leather strips. All samples were dried at 60° C. for  $\frac{1}{2}$  hour between coats and subjected to a similar drying period after the second coat and then cooled for 3 hours at a temperature of 20 24.5° C. and a relative humidity of 31%.

Pairs of uncoated and coated leather strips with the coated surfaces held together under moderate pressure with flexible rubber bands were suspended in a high frequency electrostatic field of 25 30 megacycles per second and an applied input voltage to the oscillator of 2100 volts for a period of 45 seconds and the rise in temperature determined as in Example 1.

The following averaged results were obtained:

|                                               | Temperature reached | Rise above room temperature |
|-----------------------------------------------|---------------------|-----------------------------|
| Leather strips—no coating                     | 66.0                | 41.5                        |
| Leather strips with coating free of rutile    | 71.0                | 46.5                        |
| Leather strips with coating containing rutile | 76.5                | 52.0                        |

40 Further illustrative of the novel and desirable effects afforded by the use of rutile for inducing heat in organic dielectric materials are the power absorption results obtained by testing sheets of 45 polymerized methyl methacrylate. Two sheets of this material 1 1/2" x 3" and 1/8" in thickness and held together with flexible rubber bands were suspended in a high frequency field of 30.6 megacycles per second and an impressed input voltage to the oscillator of 2100 volts. Power absorption was found to be 21 watts. This test was repeated 50 with a layer of rutile amounting to about 50% of the weight of the sheets uniformly interposed between the two sheets of polymerized methyl methacrylate resin and in this case the power absorption was 63 watts.

55 As indicated above, titanium dioxide in the rutile or brookite form is preferred in the operation of the present invention because of their unusually high dielectric constants. The anatase form with its relatively low dielectric constant fails to provide the advantages of the rutile and brookite forms and, therefore, is of little use as a means for increasing the hysteresis losses in the polymeric organic materials herein described.

60 65 It has been found that an amount of rutile or brookite of between about 20 to 50% by weight of the total solids of the composition to be treated gives improved results with about 30 to 40% by weight of the total solids giving greatest improvement.

65 70 The invention is of general utility for inducing heat in organic polymeric materials when such materials are exposed to energized electrostatic fields of radio frequencies, preferably frequencies between about 100,000 cycles and 100

megacycles and especially at frequencies of about 30 megacycles, these frequencies having been found most useful in treating such materials. As already suggested, an important use resides in the field of cementing operations where the parts to be joined are coated with an organic adhesive and then activated by heat induced in the adhesive by an energized high frequency electric field. The incorporation of the specific agents described above in synthetic resinous materials in the monomeric or unpolymerized state including phenolic, urea aldehyde, acrylic acid resins, alkyd and styrene type resins promotes the heating of such materials when exposed to high frequency electrostatic fields thereby converting them to the polymeric state. The agents are also useful in cellulose derivative compositions containing cellulose nitrate, cellulose acetate, cellulose ethers and mixed cellulose esters such as cellulose acetobutyrate and cellulose acetopropionate.

Of particular advantage is the increase in hysteresis losses at high frequencies occasioned by the addition of the rutile or brookite forms of titanium dioxide to organic polymeric dielectric materials. In some instances, such materials have such low losses at radio frequencies that no heating results are experienced when they are placed in an electrostatic field of such frequencies. However, the incorporation of the suggested modifying agents, even though they are excellent dielectric materials themselves, causes a change in the electrical properties of the organic material so that the hysteresis losses are increased to a point that heating results at such frequencies. The invention presents desirable advantages even with organic polymeric materials which normally respond to electrostatic fields of frequencies between 100,000 cycles and 100 megacycles in that the rate and amount of heat so induced is markedly increased.

It is apparent that many widely different embodiments of the invention may be made with-

out departing from the spirit and scope thereof and, therefore, it is not intended to be limited except as indicated in the appended claims.

I claim:

1. The process of inducing heat in organic materials of high dielectric value which comprises dispersing titanium dioxide selected from the group consisting of rutile and brookite in said organic material and placing the so modified material in an energized electrostatic field of radio frequency.

2. Process of claim 1 in which the frequency of the electrostatic field is between 100,000 cycles per second and 100 megacycles per second.

3. Process of claim 1 in which the frequency of the electrostatic field is about 30 megacycles per second.

4. In the process of heating organic monomeric and polymeric materials of high dielectric value by exposing said materials to an energized high frequency electrostatic field, the step of incorporating titanium dioxide selected from the group consisting of rutile and brookite in said organic material and thereafter placing the so modified material in an energized high frequency field, said frequency being from 100,000 cycles per second to 100 megacycles per second.

5. Process of claim 4 in which the titanium dioxide is present in an amount between about 20 and 50% by weight of the total solids.

6. Process for promoting the polymerization of unpolymerized and monomeric organic materials of high dielectric value which comprises dispersing titanium dioxide selected from the group consisting of rutile and brookite in said organic material and exposing the so modified material to an energized electrostatic high frequency field until the material is polymerized, said frequency being from 100,000 cycles per second to 100 megacycles per second.

7. Process of claim 6 in which the monomeric material is monomeric styrene resin.

CHARLES B. HEMMING.